

## 1

3,184,409

HYDROCARBON COMPOSITIONS CONTAINING  
IODINE AS AN ANTI-FRICTION AGENTMichael J. Furey, Berkeley Heights, N.J., assignor to Esso  
Research and Engineering Company, a corporation of  
DelawareNo Drawing. Filed Jan. 31, 1962, Ser. No. 170,249  
2 Claims. (Cl. 252—33)

This invention relates to compositions containing iodine. In particular, it relates to such compositions which exhibit extremely low coefficients of friction.

There are many instances, particularly under "boundary lubrication" conditions where two rubbing surfaces to be lubricated are separated by a very thin film of lubricant. In these circumstances, it is desirable that there be very little friction occurring between the moving surfaces. To reduce this friction, it has been customary to fortify conventional lubricants with additives known as oiliness agents. It has now been discovered that very small quantities of iodine within a carrier medium act as an exceptionally effective oiliness agent. Moreover, this use of elemental iodine in such carrier mediums results in significant secondary benefits, that is, improvements in load-carrying capacity and antiwear characteristics.

By oiliness agents is meant those materials which lower the coefficient of friction of certain materials, usually lubricants. Materials which prevent wear are known as antiwear agents. The two foregoing agents must be distinguished from additives which improve load-carrying capacity of lubricants. Such additives prevent the seizing and/or welding of moving surfaces (usually metal parts) and are commonly referred to as "extreme pressure" or EP agents. These latter additives may sometimes prevent wear, but oiliness and EP properties are not generally found together to an equal degree in a given additive.

The instant invention relates to the discovery that much lower concentrations of iodine than those of any previously known oiliness agent, e.g., as low as 0.0001 wt. percent, of iodine in carrier mediums, e.g., hydrocarbons, can drastically lower the coefficient of friction existing between two rubbing surfaces which contact a carrier medium having iodine dispersed or dissolved therein. For example, as low as 0.00375 wt. percent of iodine in a mineral oil carrier medium can lower the coefficient of friction more than 50%. Suitable carrier mediums can be represented by hydrocarbons such as lubricating oils, organic liquids such as benzene, xylene, etc. In special circumstances, aqueous media, water, liquid emulsions and other fluid mediums such as air, inert gases and other gases can be used.

The hydrocarbons are the preferred carrier mediums. Preferably the hydrocarbons should not include highly reactive species. The preferred hydrocarbons are paraffins, naphthenes and aromatics, with the paraffins and naphthenes most preferred, e.g., the compositions should contain at least 50% saturated hydrocarbons and at most 50% aromatics and not more than 20% of other unsaturated hydrocarbons such as olefins or cycloolefins.

Suitable hydrocarbons are those occurring naturally in petroleum and particularly those used for lubrication of machinery, e.g., neutral oils having viscosity between 50 SUS at 100° F. and 2000 SUS at 100° F. or bright stocks having a viscosity between 90 and 300 SUS at 210° F. But any petroleum product which is required to have oili-

## 2

ness in certain uses can be improved in this property by adding iodine, e.g., solid products like paraffin wax, semi-solid products like petrolatum and greases, or relatively non-viscous products like kerosene and gas oil or fuel oil. The preferred petroleum hydrocarbons are those boiling above 300° F. and especially preferred are those boiling above 500° F. at atmospheric pressure.

For many of the ordinary applications of the invention, lubricating oils, cutting oils, metal working oils, hydraulic fluids, pneumatic equipment oils, spindle oils, gear oils, and the like will be used as the carrier medium for the iodine. It is contemplated that the lubricating oils which are to be used as carrier mediums include straight mineral lubricating oils or distillates derived from paraffinic, naphthenic, asphaltic, or mixed base crudes or, if desired, various blended oils can be employed as well.

Of course, synthetic lubricating oils made from esters, polysiloxanes, carbonates, formals, polyglycols, and the like can also be used. Also mixtures of synthetic and mineral oils can be employed. However, there are other more specialized applications in which it is not necessary that conventional oil bases be utilized to carry iodine. Iodine crystals can be placed in sealed systems to provide lubrication as they gradually sublime. In this technique, the particular gas which happens to be in the sealed system provides a carrier medium. This latter application can be seen to be of particular significance for lubricating rocket or missile systems where the rubbing surfaces can be sealed and the circulating iodine will provide the necessary lubrication.

Moreover, it has been discovered that the exposure of metal lubricating or rubbing surfaces to iodine results in a beneficial carryover effect. This means that the low frictional effect on rubbing surfaces will last for a time after that in which the surfaces are removed from the presence of iodine. Thus, the low frictional effects caused by the iodine can exert their protective effect even after the carrier medium containing iodine is removed from the system. The carryover effect can be of significant value in certain specialized applications. For instance, when rubbing surfaces are exposed to iodine, then at a later date in the absence of any lubricant, these same rubbing surfaces can be brought into rubbing contact with each other without causing excessive friction. This aspect of the invention can be particularly important when the weight of the lubricant is a critical factor. This weight factor is of great importance in a rocket missile system. For instance, in such a system a fluid carrier medium can be chosen without regard to its inherent lubrication values and only with regard to its coolant properties. Thus, a portion of the liquid fuel from the rocket and missile fuel system could be used as a carrier medium which obviously would not add extra weight to the system.

Aqueous solutions containing iodine or iodine complexes are effective metal working fluids or specialty lubricants (e.g., where nonflammability is desired). These solutions can be used in cutting, grinding, machinery, threading, tapping, wire drawing, extrusion, or any other metal working operation in which low friction, low tool wear, faster processing or better surface finish is desired. Since iodine is known to react with titanium, particularly at higher temperatures, these solutions are suitable for machining titanium as well as other metals and alloys normally considered difficult to work with.

Iodine is less soluble in water than in most organic sol-

vents. For example, at 25° C., the solubility of iodine in n-hexane is about 1.3%, in water it is about 0.034%. Iodine is quite soluble in aqueous iodide solutions, however, owing to the formation of polyiodide ions. Some of these solutions are very concentrated; for example, that in equilibrium with iodine and KI, 7H<sub>2</sub>O at 25° C. contains about 68% iodine, 25% potassium iodide and 7% water. (Iodine is also more soluble in solutions of chlorides, bromides, and other salts in water, although these salts have less effect than the iodides.)

Another interesting, and useful, property is that solutions of iodine in water are hydrolyzed to a much smaller extent than those of other halogens. The equilibrium constant for the reaction:



is only about  $5 \times 10^{-15}$  at 25° C. An aqueous solution containing iodide, iodate, and free iodine or triiodide ion, has a pH of just about 7.

Suitable aqueous metal working solutions containing iodine are:

- (1) Iodine alone dissolved in water.
- (2) Iodine in combination with inorganic iodides such as KI dissolved in water.
- (3) Complexes of iodine with polyhydric compounds dissolved in water. The polyhydric compounds would include starches, amylose, amylopectin, sorbitols, polyethylene glycols and any other compounds containing an appreciable number of OH groups. (Polyols are preferred to glycols.)
- (4) Combinations of any of those listed above.

Other additives can also be incorporated in any of the above solutions. These include corrosion inhibitors (e.g., nitrites, chromates, phosphates, imidazolines, sulfonates, amines), wetting agents, thickeners and dyes. Mutual solvents such as alcohols or ethers can also be incorporated.

For many practical applications conventional lubricating fluids, e.g., petroleum oils, hydrocarbons and organic fluids are the preferred carrier medium. In other applications fuels will be a preferred carrier medium. In such carrier mediums, the overall final composition will desirably comprise a major proportion of fluid and 0.0001 to 0.99, preferably 0.001 to 0.90 of iodine by weight. All percentage concentrations referred to herein are by weight and are based on the weight of the finished formulation. In other carrier mediums such as aqueous media the concentration of iodine will be from 0.0001 to 5, e.g., 0.001 to 3 wt. percent.

For both types of carrier mediums, the preferred concentrations vary within narrower limits in the above ranges. Concentrations between 0.09% and 0.99% are suitable primarily as "concentrates," which in lubricating service are diluted to lower concentrations, e.g., after the initial oiliness film has been established on the metal surfaces. Concentrations between 0.0009% and 0.09% are particularly effective for providing oiliness while equilibrium conditions prevail. The most preferred concentrations are between 0.005 and 0.085% by weight.

Inasmuch as iodine tends to be lost by sublimation from a lubricated metal surface, replacement of what is thus lost may be achieved by supplying iodine in extremely dilute solution, e.g., 0.0001 to 0.009%. In a particular example, the motor oil in the crankcase of an engine can have 0.05% iodine dissolved in it initially and the supply to makeup for sublimation losses from the crankcase can be provided by adding 0.005% iodine to the fuel, e.g., gasoline in an Otto cycle engine or gas oil in a Diesel cycle engine, so that during the intake stroke of the piston in such engine the incoming fuel would replenish the iodine content of the oil film on the piston walls.

In some instances when using iodine itself in a crankcase oil some loss of iodine by vaporization may occur, particularly at the higher oil temperatures. However,

the incorporation of iodine into the fuel, rather than the lubricant, will circumvent this problem. Some dilution of the oil by the fuel always occurs and the fuel can be the source of iodine for the oil. With the relatively large amounts of fuel being utilized per unit of time, the concentrations of iodine needed in the fuel can be very low.

Thus, friction and/or wear, occurring in any fuel burning device (e.g., internal combustion engine, diesel engine, gas turbine) can be minimized or reduced by the incorporation of elemental diiodine in the fuel. The concentration range can be from 0.0001 wt. percent I<sub>2</sub> to 0.9 wt. percent I<sub>2</sub> although 0.0005 to 0.05 wt. percent I<sub>2</sub> is preferred, all wt. percent being based on the weight of the final formulation. The fuels could consist of gasoline, heating oil, jet fuel, gas oil, kerosene or any other fuel in which iodine can be incorporated.

If necessary or desirable, other additives could be used in combination with iodine in fuels for certain specific properties or to overcome any deficiencies (e.g., staining of metals). These would include sulfonates, unsaturated compounds, cyclic alcohols and the like.

Iodine can be incorporated in hydrocarbons or other liquid carrier mediums by either dissolving solid iodine in the liquid, adding a solution of iodine in a medium more volatile than the desired carrier medium and flashing off the more volatile substituent, or by bubbling iodine vapor through the desired carrier medium, e.g., a hydrocarbon.

Other additives can be added to the carrier medium composition of the present invention in order to form a finished lubricant. Such additives include oxidation inhibitors such as phenothiazine or phenyl- $\alpha$ -naphthylamine; detergent inhibitors such as the barium salt of isononyl phenol sulfide; pour point depressants such as copolymers of vinyl acetate with fumaric acid esters of coconut oil alcohols; viscosity index improvers such as polymethacrylates; and the like.

The technique of the invention is applicable to all metals used in machines and including ferrous metals such as iron and steel, nonferrous metals such as aluminum, copper, silver, cadmium, and the like, and alloys such as bronze, constantan, and the like. Furthermore, the invention is applicable to non-metals such as glass and synthetic plastics.

It has been found that when iodine is used in the higher concentration ranges, i.e., from about 0.0075 wt. percent and above, e.g., 0.009 to 0.99 particularly between 0.09 and 0.99%, some staining occurs on certain metal parts, particularly iron and steel, that are in contact with the iodine. This stain has no effect on the oiliness and other properties of the iodine composition. However, it has been found that this staining can be eliminated without affecting the otherwise desirable properties of the iodine. The elimination of such staining constitutes an additional feature of the invention.

Elemental iodine atoms or molecules in unreacted form in solution can form a loose association with other materials to form a complex. Many complexes of iodine exist. The well-known complexes include those of iodine with benzenes, ketones and ethers. Iodine also forms complexes with starch, polyhydric compounds and compounds containing a carbonyl group, as well as with nitrogen-containing compounds. These iodine complexes are useful as additives to reduce friction and wear. Materials with which iodine forms complexes useful as additives include the following specific examples:

Nitrogen containing compounds such as pyridines, picolines, quinolines, isoquinoline, quinaldine, indole, acridine, acridone, carbazoles, piperazines and the like;

Ethers such as di-n-amyl ether, divinyl ether, diphenyl ether, anisole, dibutyl "Carbitol," 2-methyl-2-ethyl-1,3-dioxolane, 2,3-epoxy-2-ethyl hexanol, styrene oxide, triisobutylene oxide, epichlorohydrin and dipentane dioxide and the like;

Alcohols such as hexanol, isoctyl alcohol, tridecyl al-

cohol, hexadecyl alcohol, eicosyl alcohol, cyclohexanol, n-decyl alcohol and benzyl alcohol and the like;

Ketones such as acetone, methyl ethyl ketone, methyl isobutyl ketone, ethyl butyl ketone, isophorone, isobutyl heptyl ketone, stearone, mesityl oxide, cyclohexanone and benzophenone, and the like;

Acids such as formic, acetic, caprylic iodoacetic, glycolic, lactic, thioglycolic, cyanoacetic, 2-ethyl hexoic, isodecanoic, naphthenic, benzoic, oleic, ricinoleic, oxo acids and C<sub>36</sub> dimer acids, and the like;

Esters such as isopropyl acetate, vinyl acetate, butyl "Cellosolve" acetate, sebacates, adipates, silicates, succinates, oleates, carbonates, and the like;

Aldehydes such as n-heptaldehyde, C<sub>8</sub>-C<sub>13</sub>-C<sub>16</sub> Oxo aldehydes, stearaldehyde, 2-methylpentaldehyde, 1,2,3,6-tetrahydrobenzaldehyde, and furfural, and the like.

Polymers having the above functional groups or combinations thereof are also suitable. Sulfonic acids and their salts are also suitable. Iodine can be mixed in suitable proportions, e.g., equimolar, with compounds of those classes and the mixtures can be dissolved in hydrocarbons. Alternately iodine and one or more compounds of those classes can be dissolved separately in the same hydrocarbon. The resulting hydrocarbon solutions of the iodine complexes retain the properties of lowering the coefficient of friction and decreasing or preventing the wear of metal surfaces in machines but said solutions do not stain said metal surfaces. For instance, in illustration of the above, the following specific compounds in the presence of the iodine will eliminate staining. These compounds as examples are a mixed 1,2 epoxyhexadecane and 1,2 epoxyoctadecane obtainable commercially as a C<sub>16</sub>-C<sub>18</sub> olefin oxide from the FMC Corp., barium sulfonate, and decyl alcohol. The above compounds are used in amounts of 50-150, e.g., 75-100, wt. percent based on the weight percent of iodine.

The use of sulfonates in connection with the iodine not only eliminates staining but also permits the attainment of good high temperature lubrication characteristics. For some types of lubrication the bulk temperature of the lubricant can reach such high temperatures so as to cause the iodine to be driven out of the carrier medium. For example, by using barium sulfonate in conjunction with iodine, adequate retention of the excellent lubricating properties of the iodine alone is accomplished. Although barium sulfonate is a preferred sulfonate other detergent additives can be used. The detergent lubricant additives which are preferred and are well known in the lubricating art include the petroleum sulfonates, synthetic alkyl aryl sulfonates, various alkyl phenates, alkyl phenate sulfides, phosphosulfurized olefin polymers, and various combinations of these additives. Following are specific descriptions of several of the above types of detergent additives.

Petroleum sulfonates generally used as lubricating oil detergents are the oil-soluble alkaline earth metal salts of high molecular weight sulfonic acids. These sulfonic acids are produced by the treatment of petroleum oils of the lubricating oil range with fuming sulfuric acid and generally have molecular weights of about 300 to 700, e.g., 350 to 500. Petroleum sulfonates are well known in the art and have been described in numerous patents, e.g., U.S. 2,467,176.

Detergent sulfonates can also be derived synthetically from relatively pure alkyl aryl sulfonic acids having from about 10 to 33 carbon atoms per molecule. For example, sulfonated products of alkylated aromatics such as benzene, toluene, xylene, and naphthalene, alkylated with olefins or olefin polymers of the type of polypropylene, polyisobutylene, etc. can be used.

Specific examples of the above two types of sulfonates include calcium petroleum sulfonate, barium petroleum sulfonate, calcium di-C<sub>8</sub> alkyl benzene sulfonate, barium di-C<sub>9</sub> alkyl benzene sulfonate and calcium C<sub>18</sub> alkyl benzene sulfonate; wherein said di-C<sub>8</sub> alkyl group is derived

from diisobutylene; said C<sub>8</sub> alkyl group is obtained from tripropylene and said C<sub>18</sub> alkyl group is obtained from tetraisobutylene.

The above sulfonates may be either neutral sulfonates, i.e., where the sulfonic acid is neutralized with an equal mole equivalent amount of metal base, or the sulfonates may be of the so-called "high alkalinity" type. In the latter case, additional metal base, in excess of that required for simple neutralization, is reacted with the sulfonate sulfonic acid to form an alkaline product which can then be blown with carbon dioxide to reduce its alkalinity and form a substantially neutral final product. Recent work has indicated that such so-called high alkalinity sulfonates are probably dispersions of neutral sulfonates and a carbonate of the metal used which are believed to exist in the form of colloidal sols. In any event, the term sulfonate as used herein and in the appended claims includes both neutral sulfonates and so-called high alkalinity (or high metal content) sulfonates.

20 The invention will be further understood by reference to the following examples which illustrate preferred forms of the invention. All percentages of the compositions of the examples are weight percentages and based on the weight of the finished composition.

#### Example I

In order to evaluate the compositions of the examples, they were tested in a rotating cylinder apparatus designed to measure metallic contact and friction between sliding, lubricated surfaces. Other noninventive compositions were also evaluated for comparison purposes. A complete description of this apparatus was given in a paper entitled, "Metallic Contact and Friction Between Sliding Surfaces" by M. J. Furey presented at the 1960 Joint 30 ASLE-ASME Lubrication Conference, October 19, 1960, in Boston, Mass. This paper has been published by the American Society of Lubrication Engineers, 5 N. Wabash Ave., Chicago 2, Illinois, under the above noted title in ASLE Transactions, volume 4, Number 1, pages 1-11, 40 April 1961. The apparatus has also been described in copending application S.N. 80,474, filed January 3, 1961, now U.S. Patent No. 3,129,580, by M. J. Furey and J. A. Wilson. The paper and copending application are here-with incorporated in their entirety in this application.

The apparatus consists basically of a fixed metal ball 45 loaded against a rotating steel cylinder. The extent of metallic contact is determined by measuring both the instantaneous and average electrical resistance between the two surfaces. It is expressed as the percent of the time that metallic contact occurs in a given period of 50 time. Friction between the ball and cylinder is recorded simultaneously with contact. This is noted as coefficient of friction which is the ratio of friction force to the load. It has been found that there is, in general, a good correlation between metallic contact measured in this manner 55 and the amount of surface damage which occurs.

The evaluations of the compositions were obtained under the following conditions unless otherwise noted:

System: AISI 52100 Steel, 1/2" diam. ball on 1 3/4" diam. 60 cylinder

Load: 240 grams (54,700 p.s.i. mean Hertz pressure)

Speed: 240 r.p.m. (56 cm./sec. sliding velocity)

Time: 32 minutes

Temperature: 77° F.

65 A solution containing 0.75 wt. percent iodine was prepared by adding elemental iodine to a solvent-extracted, paraffinic, neutral mineral oil having a viscosity of 100 SUS at 100° F. and mixing at ambient temperature. The resultant blend was clear with a dark amber color. A 70 portion of this blend was set aside and the remainder diluted to give a blend having a 0.075 wt. percent concentration of iodine. The latter blend was further diluted in the same manner and treated identically as the first blend. This procedure was carried out until there 75 were five blends containing the concentrations of 0.75

wt. percent, 0.075 wt. percent, 0.0075 wt. percent, 0.00375 wt. percent, and 0.00075 wt. percent iodine. The iodine blends and the mineral oil base alone with no additives were evaluated in the ball-on-cylinder device. The evaluation was in terms of percent metallic contact and coefficient of friction. The blends were labeled from A through F. The average results of several evaluations and the designations of particular blends are given in Table 1 following.

Table 1  
EFFECT OF IODINE ON METALLIC CONTACT AND FRICTION

Base oil: Mineral oil (100 SUS at 100° F.)  
Time: 32 minutes

| Blend | Concentration of iodine (wt. percent) | Average percent metallic contact | Average coefficient of friction |
|-------|---------------------------------------|----------------------------------|---------------------------------|
| A     | 0                                     | 85                               | 0.090                           |
| B     | 0.0075                                | 89                               | 0.090                           |
| C     | 0.00375                               | 65                               | 0.040                           |
| D     | 0.0075                                | 13                               | 0.005                           |
| E     | 0.075                                 | 1                                | 0.005                           |
| F     | 0.75                                  | 1                                | 0.020                           |

As can be seen by the above data from Table 1, the iodine has a pronounced effect in reducing friction in metallic contact. Even more remarkably, the effect occurs at a concentration of iodine as little as 0.00375 wt. percent. At 0.0075 wt. percent iodine concentration, there is a significant reduction in metallic contact and a more than 50% reduction in friction.

These effects are unusually large. For example, the average reduction in friction for blends containing 0.0075% iodine or more was 89%. The average reduction in metallic contact for the same oils was about 94%.

#### EXAMPLE II

It is well known that solutions of iodine generally fall

Table 2

#### EFFECT OF IODINE ON METALLIC CONTACT AND FRICTION

Base oil: White oil (100 SUS at 100° F.)

Time: 32 minutes

| Blend | Concentration of iodine (wt. percent) | Percent metallic contact | Coefficient of friction |
|-------|---------------------------------------|--------------------------|-------------------------|
| G     | 0                                     | 82                       | 0.105                   |
| H     | 0.00375                               | 0                        | 0.005                   |
| I     | 0.0075                                | 9                        | 0.005                   |
| J     | 0.075                                 | 0                        | 0.020                   |
| K     | 0.75                                  | 11                       | 0.020                   |
| L     | 1.00                                  | 3                        | 0.020                   |
| M     | 1.25                                  | 1                        | 0.020                   |

As can be seen by the above Table 2, the results obtained with iodine in a white oil are quite outstanding. On the average, iodine reduces metallic contact and friction by about 95% and 85% respectively in these tests.

#### EXAMPLE III

In order to determine the effectiveness of various additives in preventing metal staining by the iodine, a series of four blends was prepared. One blend was the base oil of Example I; one blend was the same base oil plus 0.85 wt. percent iodine and the other two blends were the base oil plus 0.85 wt. percent iodine plus 1 wt. percent each of a series of additional additives. The question to be determined was whether or not these compounds could reduce staining and, if they reduced staining, would they have any adverse effect on the ability of iodine to reduce contact and friction. The blends, as described above, were labeled N through S. Each test piece was then immersed in 50 cc. of the oil blend for 72 hours at room temperature. In this test, the test ball was an AISI 52100 steel 1/2 inch test ball and the time of testing was 72 hours at room temperature. The results of the test and the designation of the blends are summarized below in Table 3.

Table 3

#### EFFECT OF IODINE AND OTHER ADDITIVES ON STAINING, METALLIC CONTACT AND FRICTION

Base oil: Neutral mineral oil (100 SUS at 100° F.)

| Blend | Oil                                                      | Dark stain? | Percent metallic contact | Coefficient of friction |
|-------|----------------------------------------------------------|-------------|--------------------------|-------------------------|
| N     | Neutral mineral oil                                      | No          | 85                       | 0.090                   |
| O     | Mineral oil+0.85% iodine                                 | Yes         | 3                        | 0.004                   |
| P     | Blend O+1% C <sub>15</sub> -C <sub>18</sub> olefin oxide | No          | 9                        | 0.002                   |
| Q     | Blend O+1% barium sulfonate                              | No          | 0                        | 0.002                   |
| R     | Blend N+3% Cd naphthenate                                | No          | 88                       | 0.090                   |
| S     | Blend R+0.85% iodine                                     | No          | 84                       | 0.050                   |

into two main classes, amber and violet. In Example I above it was observed that the blends of iodine in the 100 SUS mineral oil were various shades of amber. It had been observed that when iodine blends were prepared in white oil, the blends had a violet color. Therefore, to determine whether the form in which the iodine was present had any influence on metallic contact and coefficient of friction, ball-on-cylinder tests were carried out with blends of iodine in a white oil which was a highly refined mineral oil. This white oil had a viscosity of 100 SUS at 100° F. and is obtainable commercially as Marcol JX from the Humble Oil & Refining Co. The method of preparation and evaluation was similar to that described in Example I. White oil alone without iodine or other additives was used as a control. The blends were labeled from G through M. The results (average) of the tests and the designations of the blends are summarized below in Table 2.

As can be seen by the above table, the additives in the iodine blend completely eliminated dark stain.

The barium sulfonate used in the above test was "Hybase" barium sulfonate obtained from Bryton Company and prepared by the carbonation process previously described.

Thus, the inclusion of iodine in a carrier medium such as a lubricating oil results in a reduction of metallic contact and a lowering of the coefficient of friction far beyond that obtainable with ordinary additives. For instance, a typically effective material of the prior art for reducing friction under conditions similar to those of the above examples was one weight percent of isopropyl oleate. It reduced friction by about 50%. Moreover, other conventional antiwear additives such as oleic acid, tricresyl phosphate, metal thiophosphates, such as zinc dialkyl dithiophosphate, halogen E.P. additives and the like at best reduce friction by no more than about 30%.

9  
EXAMPLE IV

In order to evaluate the iodine-containing compositions with similar compositions containing other halogens, e.g., gromine, the following procedure was carried out. Blends D, E, and F were compared in the ball-on-cylinder apparatus with three identical blends except that bromine was used in place of iodine. Blend A was used as the base oil. It is to be noted that in performing these tests in this and other examples, a new ball is used with each new portion of the cylinder. Thus, a new ball and fresh cylinder track was used for each run with a given additive. For a given additive, tests were started with the base oil, then the lowest concentration, and so on—using one cylinder. Different additives were tested on different cylinders, however. All the  $I_2$  data below were obtained on one cylinder and all the  $Br_2$  data were obtained on another. (A new ball and fresh track were used for each test.) This accounts for the variations in test results wherein the figures for metallic contact and coefficient of friction vary with respect to the same base oil. The results of the evaluation are summarized in Table 4 below.

Table 4

| Halogen                                                              | Percent metallic |        | Coefficient of friction |        |
|----------------------------------------------------------------------|------------------|--------|-------------------------|--------|
|                                                                      | $I_2$            | $Br_2$ | $I_2$                   | $Br_2$ |
| Wt. percent in neutral lube oil having a vis. of 100 SUS at 100° F.: |                  |        |                         |        |
| 0                                                                    | 85               | 72     | 0.090                   | 0.090  |
| 0.0075                                                               | 13               | 40     | 0.005                   | 0.040  |
| 0.075                                                                | 1                | 26     | 0.005                   | 0.030  |
| 0.75                                                                 | 1                | 100    | 0.020                   | 0.090  |

The above table demonstrates that iodine decreases metallic contact and coefficient of friction to a much greater extent than bromine under identical conditions.

## EXAMPLE V

In order to evaluate the compositions of the invention, Blends D, E, and F, and I, J, and K were tested in an S.A.E. machine and a shell 4-ball E.P. test. These are well-known tests in the lubricating art.

The results of these tests are summarized in Table 5 which follows.

Table 5

## EXTREME PRESSURE PROPERTIES OF MINERAL OILS CONTAINING IODINE

| Lubricant                            | S.A.E. machine load carrying capacity lbs. | 4-ball E.P. test  |                  |
|--------------------------------------|--------------------------------------------|-------------------|------------------|
|                                      |                                            | Seize point (kg.) | Weld point (kg.) |
| Neutral solvent extracted distillate | 1<100                                      | 63                | 100              |
| +0.0075% $I_2$                       | 1<100                                      | 56                | 100              |
| +0.075% $I_2$                        | 1<100                                      | 100               | 141              |
| +0.75% $I_2$                         | 4,000                                      | 178               | >355             |
| White oil                            | 1<100                                      | 36                | 89               |
| +0.0075% $I^2$                       | 1<100                                      | 45                | 100              |
| 0.075% $I_2$                         | 2,600                                      | 112               | 178              |
| +0.75% $I_2$                         | 3,800                                      | 141               | >355             |

<sup>1</sup> Failed in less than 5 seconds during break-in.

<sup>2</sup> Test discontinued at this load with no welding.

The above tests demonstrate that iodine in concentrations as high as 0.5 wt. percent begins to show some load carrying capacity. This would be expected from the prior art teachings on halogens in general. However, in the

## 10

lower, especially preferred, concentrations of the present invention the load carrying capacity is not very significant. Therefore, at the preferred concentrations of the invention, load carrying properties are minimal but the property of decreasing the coefficient of friction is at a maximum.

## EXAMPLE VI

Blend J containing 0.075 wt. percent iodine was evaluated in the ball-on-cylinder apparatus which was identical to the test conditions previously described in Example I except that the speed was 240 r.p.m. and the load in grams was respectively 240, 960, and 4000. The results of this evaluation are summarized in Table 6 below.

15  
Table 6  
EFFECT OF IODINE ON WEAR WITH STEEL AT HIGHER LOADS

20 Ball-on-cylinder tests  
AISI 52100 Steel (unhardened)  
Base oil: white oil  
Time: 32 minutes  
Speed: 240 r.p.m.

| Load (grams) | $I_2$ in oil <sup>1</sup> | Wear scar diameter on ball (mm.) |      |
|--------------|---------------------------|----------------------------------|------|
|              |                           | No.                              | Yes. |
| 240          | No.                       | 0.48                             | 0.26 |
| 240          | Yes.                      | 0.26                             | 0.78 |
| 960          | No.                       | 0.34                             | 0.80 |
| 960          | Yes.                      | 0.80                             | 0.48 |
| 4,000        | No.                       | 0.48                             | 0.48 |
| 4,000        | Yes.                      | 0.48                             | 0.48 |

<sup>1</sup> 0.075% by weight.

35 The above data show that a 0.075 wt. percent blend of iodine in white oil decreases wear over a range of loads between 240 and 4000 grams by about 50% regardless of the load.

## EXAMPLE VII

Blend J was again evaluated in the ball-on-cylinder test at 240 r.p.m. and at a 240-gram load except that the metals contacting each other varied. In the first test, the metals contacting each other were steel-on-steel. In the second test, they were bronze-on-steel. In the third test they were silver-on-steel; in the fourth, constantan-on-steel. The results of these tests are summarized below in Table 7.

50  
Table 7  
EFFECT OF IODINE ON WEAR WITH VARIOUS METAL-ON-STEEL SYSTEMS

55 Base oil: White oil  
Ball-on-cylinder tests at 240 r.p.m. and 240 g. load  
Time: 32 minutes

| System                      | $I^2$ in oil <sup>1</sup> | Wear scar diameter on ball (mm.) |      |
|-----------------------------|---------------------------|----------------------------------|------|
|                             |                           | No.                              | Yes. |
| Steel-on-steel <sup>2</sup> | No.                       | 0.48                             | 0.26 |
| Steel-on-steel <sup>2</sup> | Yes.                      | 0.95                             | 0.64 |
| Bronze-on-steel             | No.                       | 0.91                             | 0.69 |
| Bronze-on-steel             | Yes.                      | 0.69                             | 0.69 |
| Silver-on-steel             | No.                       | 0.69                             | 0.69 |
| Silver-on-steel             | Yes.                      | 0.21                             | 0.21 |
| Constantan-on-steel         | No.                       | 0.69                             | 0.69 |
| Constantan-on-steel         | Yes.                      | 0.21                             | 0.21 |

<sup>1</sup> 0.075% by weight.

<sup>2</sup> AISI 52100 steel (unhardened).

70 In each case, iodine significantly reduced wear, the actual reduction varying from about 24% (silver-on-steel) to 69% (constantan-on-steel). This demonstrates that the type of metals contacting each other is relatively unimportant. Thus, excellent results are obtained when different metals contact each other.

Blend J was evaluated in the ball-on-cylinder test where the metals contacting each other were both aluminum. The test was carried out over a range of loads consisting of 240 grams, 960 grams, and 4000 grams. The results of this test are summarized below in Table 8. 5

Table 8

## EFFECT OF IODINE ON LUBRICATION OF ALUMINUM-ON-ALUMINUM

Base oil: White oil  
Ball-on-cylinder tests at 240 r.p.m.  
Time: 32 minutes

| Load (gms) | I <sup>2</sup> in oil <sup>1</sup> | Percent metallic contact | Coefficient of friction | Wear scar (mm.) |
|------------|------------------------------------|--------------------------|-------------------------|-----------------|
| 240        | (No)                               | 91                       | 0.09                    | 0.36            |
|            | (Yes)                              | 39                       | 0.041                   | 0.48            |
| 960        | (No)                               | 248                      | <sup>2</sup> 1.89       | 0.87            |
|            | (Yes)                              | 92                       | 0.01                    | 0.63            |
| 4,000      | (No)                               | 86                       | 0.12                    | 1.25            |
|            | (Yes)                              | 88                       | 0.04                    | 0.74            |

<sup>1</sup> 0.075% by weight.<sup>2</sup> Scuffing and chattering occurred during this test (excessive bouncing probably explains 48% metallic contact).

The above data demonstrate that the compositions of the invention provide a low coefficient of friction and low wear in an aluminum-on-aluminum system. 15

## EXAMPLE VIII

Blend F was evaluated in a V-8 Chevrolet engine at 3000 revolutions per minute and at an oil sump temperature of 20° F. The purpose of this test was to measure the frictional horsepower and improvement in fuel consumption over conventional motor oils in an actual engine. Blend F was compared in this test with the base mineral neutral oil having a viscosity at 100° F. of 100 SUS and with a commercial type motor oil having a viscosity of 12.4 centistokes at 210° F. Other test conditions of this engine were a brake h.p. of 52, a water jacket temperature of 180° F.  $\pm$  3 and an air intake temperature of 110° F.  $\pm$  5. The engine was placed on a dynamometer test stand and the torque that was required to operate it was both measured and recorded with a strain gauge system. The system was so equipped that at any time during the running of the engine the friction could be measured. The system also was equipped with a measured sight glass containing fuel which could be used to determine the fuel consumption of the engine during its operation. The technique employed in this test is fully described in a paper entitled, "The Effect of Lubricant Viscosity and Composition on Engine Friction and Bearing Wear" by E. H. Okrent which was published in the ASLE Transactions, volume 4, Number 1, April 1961. The specific details of this technique are given on page 98 of this publication. The results of this test are summarized below in Table 9. 20

Table 9

## EFFECT OF IODINE ON ENGINE FRICTION

|                                                             | Frictional H.P. | Percent improvement in fuel consumption over test with regular motor oil <sup>1</sup> |
|-------------------------------------------------------------|-----------------|---------------------------------------------------------------------------------------|
| Regular motor oil (12.4 cs./210° F.)                        | 25.0            | 0                                                                                     |
| Neutral lube oil (4.2 cs./210° F.)                          | 24.0            | 1.3                                                                                   |
| Neutral lube oil +0.75% I <sub>2</sub> after operation for: |                 |                                                                                       |
| 119 min.                                                    | 22.8            | 4.0                                                                                   |
| 179 min.                                                    | 21.8            | 4.2                                                                                   |
| 277 min.                                                    | 21.5            | 4.5                                                                                   |
| 376 min.                                                    | 21.0            | 5.2                                                                                   |

<sup>1</sup> Based on indicated H.P. which is the sum of the friction H.P. and brake H.P. (in this case 52).

The above data show that approximately a 12% reduction in frictional H.P. in a Chevrolet V-8 engine as well as a 5% reduction in fuel consumption as compared with a regular motor oil was attained with 0.75% iodine dissolved in the oil. With the mineral oils alone, the friction H.P. remains constant with time.

While the above invention has been described with some particularity, it is to be understood that minor modifications can be made while still retaining the spirit and scope of the invention as hereinafter claimed.

What is claimed is:

1. A lubricating oil composition comprising a major proportion of a mineral lubricating oil and a friction-reducing amount, within the range of 0.0009 to 0.09 wt. percent, of iodine.

2. A composition according to claim 1, in which said iodine has a tendency to stain iron, and a material complexed with said iodine having the ability to reduce said tendency to stain, said material being selected from the group consisting of barium sulfonate, cadmium naphthenate, and oleic acid.

## References Cited by the Examiner

## UNITED STATES PATENTS

2,771,348 11/57 Meguerian \_\_\_\_\_ 44—79X  
3,115,467 12/63 Denison et al. \_\_\_\_\_ 252—58

## FOREIGN PATENTS

1,252 6/55 Great Britain.  
5,256 10/97 Great Britain.  
503,313 4/39 Great Britain.

## OTHER REFERENCES

Davey: "The Extreme Pressure (E.P.) Lubricating Properties of Some Bromine and Iodine Compounds, etc." J. Inst. Petrol.; 33, 673 (1947), pp. 673-677 pertinent.

Forbes: "Lubrication of Industrial and Marine Machinery," Wiley & Sons, Inc., 1943, pp. 231-235, 250-256 pertinent.

Peterson et al.: "Factors Influencing Friction and Wear With Solid Lubricant," Lubrication Eng., September-October 1955, pp. 325-330 pertinent.

60 DANIEL E. WYMAN, Primary Examiner.